

# United States Patent Office

2,849,349

Patented Aug. 26, 1958

1

2,849,349

## PROCESS FOR THE ELECTROLYTIC DEPOSITION OF ALUMINIUM

Karl Ziegler and Herbert Lehmkuhl, Mulheim an der Ruhr, Germany; said Lehmkuhl assignor to said Ziegler

No Drawing. Application July 11, 1955  
Serial No. 521,424

Claims priority, application Germany July 28, 1954

23 Claims. (Cl. 204—14)

This invention relates to a process for the electrolytic deposition of aluminium.

The problem of electrolytically depositing aluminium under gentle temperature conditions and with a low current consumption has not so far been solved satisfactorily.

The production of aluminium on a technical scale exclusively makes use of melt electrolysis at 800–900° C. in an electrolyte consisting mainly of molten cryolite. The current consumption is about 24 kilowatt hours per kilogram of aluminium.

The same process is used in principle in the electrolytic refining treatment in the so-called "three layer process." The current consumption is somewhat lower, but nevertheless is still 20 kw.-h./kg.

A series of electrolytes have been proposed for electrolysis at relatively low temperatures, but none of these, however, have actually been used in practice.

In addition to certain complex compounds of aluminium chloride with organic bases, such as pyridine, the literature has referred to certain purely inorganic electrolytes, such as, for example, sodium-aluminium chloride, in the melt or also more recently a complex aluminium compound which is formed from lithium hydride and aluminium chloride in ethereal solution (D. E. Couch and A. Brenner, Journal Electrochemical Society 99 (1952), 234).

There has not so far been any disclosure concerning the use of such electrolytes on a technical scale.

It has now been found that under certain conditions, excellent electrolytes for the deposition of aluminium under gentle temperature conditions can be synthesised from true organic aluminium compounds i. e. from such compounds which contain at least one carbon atom directly bonded to aluminium.

Aluminium trialkyls, aluminium dialkyl hydrides  $AlR_2H$ , aluminium alkyl halides, such as  $AlR_2Cl$ ,  $AlRCl_2$ , and similar substances are all non-conductors of electric current. However, they can be transformed into electrolytes by converting them into complex compounds, for example sodium ethyl with aluminium triethyl forms sodium-aluminium tetraethyl  $NaAl(C_2H_5)_4$ . In molten form, this substance has very good conductivity. This has already been shown by F. Hein (Zeitschrift für anorganische Chemie, 141, 161–226 (1924)), who obtained an oily product from sodium ethyl and aluminium triethyl and investigated it concerning its conductivity; it is true that he designated this product as being a solution of sodium ethyl in aluminium triethyl, but, as is known for certain at the present time, this product was the complex compound just referred to. F. Hein did not indicate which element is deposited on the cathode in the electrolysis. If this is investigated, it is found that mainly sodium is formed on the cathode. In addition, some aluminium may also be deposited, and spongy mixtures of sodium and aluminium are frequently observed to form at the cathode. The ratio between the amounts of sodium and aluminium which are formed

2

is dependent on the current density. It is mainly aluminium which appears with very low current densities, but aluminium is never exclusively obtained with current densities which can be used on a technical scale. This electrolyte therefore cannot be used for the deposition of aluminium. Similar remarks apply as regards a number of other such organic complex compounds, for example  $KAi(C_2H_5)_2Cl_2$  and  $NaAl(C_2H_5)_3F$ .

Excellent electrolytes of high specific conductivity for the deposition of metallic aluminium are, however, always obtained if electrolytes are used which also contain an excess of the organic aluminium compounds in addition to such complex compounds. Such electrolytes or electrolyte mixtures can not be produced as required, perhaps by combining aluminium triethyl with an one of the aforementioned complex compounds, in every case since frequency two basically possible components of such a mixture are actually not homogeneously miscible with one another. For example, a homogeneous mixture or solution can not be produced from the aforementioned sodium-aluminium tetraethyl and aluminium triethyl, since the two substances are in practice completely insoluble in one another. On the other hand, in all the combinations in which a sufficient mutual miscibility or solubility exists, it is also possible to observe that pure aluminium of excellent quality is deposited during the electrolysis.

Electrolytes which have proved to be particularly suitable are homogeneous melts of true organic aluminium compounds of the general formula  $AlR(R')_2$ , in which R represents an alkyl radical and R' represents an alkyl radical or a hydrogen or halogen atom, together with complex compounds thereof with alkali metal compounds of the general formula  $MeR'$ , wherein Me represents an alkali metal, or quaternary ammonium compounds.

Alkali metal compounds which are particularly suitable for forming the complex are alkali metal alkyls, hydrides and halides, and also tetraethyl ammonium halides, triethyl-n-butyl-ammonium halides, ethyl-tri-n-butylammonium halides, dodecyl-tri-methyl-ammonium halides, such as the chloride, and also quaternary pyridinium, quinolinium and isoquinolinium salts, such as pyridinium methiodide.

The electrolytes can be homogeneously melting compounds of true organic compounds of the general formula  $AlR(R')_2$ , in which R represents an alkyl radical and R' represents an alkyl radical or a hydrogen or halogen atom, and their complex compounds with alkali metal compounds of the general formula  $MeR'$ , wherein Me represents an alkali metal, or with quaternary ammonium compounds.

As homogeneous melts, it is also possible to use mixtures of true organic compounds of the general formula  $AlR(R')_2$ , in which R which represents an alkyl radical and R' represents an alkyl radical or a hydrogen or halogen atom, and their complex compounds with alkali metal compounds of the general formula  $MeR'$ , wherein Me represents an alkali metal, or with quaternary ammonium compounds, or homogeneously melting solutions of these substances.

For example, a suitable electrolyte is obtained by dissolving 1 mol of sodium-aluminium diisobutyl dihydride— $Na(Al-(iso-C_4H_9)_2H_2)$ —in aluminium triethyl. The basic complex compound is obtained very easily by adding sodium hydride to diisobutyl aluminium hydride. Conversely, it is obviously also possible to obtain the same electrolyte from sodium-aluminium triethyl hydride and diisobutyl aluminium hydride, or even more simply by dissolving sodium hydride in a mixture of aluminium triethyl and diisobutyl aluminium hydride.

Organic aluminium complex compounds containing fluorine have proved to be particularly suitable for com-

bining to give electrolytes of the type referred to. For example, the sodium-aluminium triethyl fluoride



with 2 mols of aluminium triethyl forms a novel and well-defined second complex compound with the composition  $\text{NaF} \cdot 2\text{Al}(\text{C}_2\text{H}_5)_3$ ; this compound is described in a prior application of the applicants and melts at a very low temperature. The specific conductivity of the melt is as follows:

$3.3 \times 10^{-3} \text{ ohm}^{-1} \text{ cm.}^{-1}$  at  $24^\circ \text{ C.}$  and  
 $15.0 \times 10^{-3} \text{ ohm}^{-1} \text{ cm.}^{-1}$  at  $80^\circ \text{ C.}$  and  
 $42.5 \times 10^{-3} \text{ ohm}^{-1} \text{ cm.}^{-1}$  at  $160^\circ \text{ C.}$

and yields by electrolysis a dense firmly adhering aluminium of excellent quality. Similarly, an electrolyte can be produced by dissolving sodium fluoride in a mixture of aluminium trimethyl and aluminium triethyl. In this case, it is again a question of the formation of a complex compound of 1 mol of sodium fluoride with 2 mols of aluminium trialkyls (which are here different from one another).

In the electrolyte mixtures to be described, it is at present not possible to indicate which complex separate compounds are actually present in the liquid electrolyte.

An example of an excellent electrolyte is one which has exactly or substantially the following composition in the melt:



Having regard to the course of the following reactions:



and



it can also be written as:



as can easily be seen by its decomposition into



This electrolyte can be produced by melting together sodium fluoride, aluminium triethyl and aluminium diethyl fluoride. Another excellent electrolyte of this group is formed if finely powdered dry cryolite is boiled with more than 6 mols of aluminium triethyl. The cryolite enters into solution. Two layers are formed, the upper layer consisting of aluminium triethyl, which can easily be separated while the lower layer has the composition:



Similar electrolytes are set out in the following table. The compositions set out therein do not have to be exactly fulfilled, but only approximately. The formulae in the table are written in such a way that it can be seen from what basic substances the electrolytes are formed. If it were desired for all formulae to be correctly expressed in the chemical sense, it would be necessary in every case for 1 mol of the alkali halide, alkyl or hydride present in the electrolyte to be combined with 1 mol of the organic aluminium compound to form a complex of the



type. It will be seen from the formulae of the electrolytes indicated below that in all cases 1 mol of the organic aluminium compound is available for each mol of alkali halide, alkyl or hydride, thus conforming to the principle of the process of the invention:



By selecting suitable quaternary ammonium salts, it is possible to produce any desired solutions of the quaternary salts in aluminium triethyl. In such electrolyte combinations, liquid phases of the predetermined composition of one salt molecule and two aluminium trialkyl molecules often do not form. It is then possible with a very wide range of variation to produce solutions which contain only a small amount of electrolyte and a large amount of aluminium triethyl.

Many of the aforementioned electrolytes can be mixed as desired or to a limited degree with solvents. The only solvents which can be used are those which do not decompose the organic aluminium compounds, for example hydrocarbons, especially those of aromatic nature. Ethers and tertiary amines, such as tetrahydrofuran, dimethyl aniline, dioxane and pyridine can also be used.

It is not recommended that the dilution of the electrolytes by such solvents should be carried too far, since then the specific conductivity is lowered and consequently a higher consumption energy is required for deposition of the aluminium. Such dilution, may, however, be advisable for protecting the electrolytes, which are very sensitive to air. Moreover, the nature and amount of solvent which is used have an effect on the properties of the deposited aluminium, especially as regards the density and hardness of the coatings.

Moreover, by using suitable solvents, it is possible to produce electrolyte combinations which are not possible without solvents owing to limited miscibility and solubility, for example the combination of sodium-aluminium tetraethyl and aluminium triethyl in the presence of some toluene.

Since the conductivity of the electrolytes rises sharply with the temperature, electrolysis temperatures higher than  $100^\circ \text{ C.}$  and up to a maximum of  $200^\circ \text{ C.}$  have frequently proved to be desirable, even if not necessary. High-boiling aromatic substances, such as methyl naphthalene, diphenyl ether and tetraline, are suitable as diluents in such cases.

If the operation is carried out without diluents, which is frequently advantageous, the heated melts of the electrolytes can be very easily protected against the action of air by covering them with a small amount of paraffin oil. They are not all miscible with paraffin oil. However, even while observing this precautionary measure, it is advisable to carry out the electrolysis processes in closed vessels and to fill the free space above the oil with an inert protective gas, such as nitrogen.

It is further to be mentioned that obviously several of the aforementioned electrolytes can also be mixed with one another in suitable manner; for example, certain amounts of sodium aluminium tetraethyl can also be dissolved in the  $\text{NaF} \cdot (\text{Al}(\text{C}_2\text{H}_5)_3)_2$  electrolyte without impairing the usefulness of the electrolyte. The excess of aluminium triethyl which even then is still present, is sufficient. The electrolytes enumerated in detail and by way of example contain methyl, ethyl and 1-butyl as organic radicals bonded to aluminium. It is obvious that a large number of similarly usable electrolytes can also be produced by using other alkyl radicals and also by using those having a higher number of carbon atoms.

This may offer certain advantages, since the sensitivity to air and especially the capacity for spontaneous ignition decreases with the large alkyl radicals. However, it will be understood that as the organic portion of the electrolyte systems becomes greater, the specific conductivity values must drop, since altogether there are fewer

ions per unit of volume. Consequently, the change-over to such higher alkyl compounds usually does not offer any particular advantages. Nevertheless, exceptions to the rule are obtained when the costs of the electric energy to be used are not important, as for example, when producing thin aluminium covering layers on wires.

The novel electrolytes can be used with advantage in all cases where it is important that a very pure aluminium should be deposited, i. e. they can be used for the production of aluminium coatings, possible on other metals such as copper, or also on a foundation material of less pure aluminium, or also for refining aluminium. In all cases, the electrolysis is preferably carried out using aluminium anodes.

In these cases, practically no losses of electrolyte occur, providing that the current density remains below about 2 am./dm.<sup>2</sup>. On the other hand, if the operation is carried out with anodes of copper, iron or platinum, for example, gas is evolved at the anodes. When the electrolytes contain the ethyl radical, the gases consist of mixtures of ethane and ethylene, and in such a case the aluminium trialkyl added in excess to the electrolyte gradually becomes exhausted during the electrolysis. Obviously, it is possible to compensate for this by adding the necessary amounts of the organic aluminium compound from time to time. When using aluminium anodes, a similar evolution of gas only becomes apparent at a high current density. Otherwise, normally the amount of aluminium which dissolves at the anode is that which has been deposited at the cathode.

If an ordinary foundry aluminium is used as anode, the impurities of the aluminium remain undissolved in the form of a black sludge. The sludge initially remains loosely clinging to the anode, but usually becomes detached during the electrolysis and falls to the bottom of the cell, but frequently also remains suspended in the electrolyte to some extent, with the possible result that particles of the anode sludge adhere to the cathode coatings and impair the deposition thereon.

This difficulty can be overcome in a very simple manner by surrounding the anodes by a tightly fitting bag of an ordinary cotton fabric, whereby the anode sludge is completely held back. Such protective devices for the anode surprisingly have an extraordinarily long effective life, despite the relatively high temperatures of the electrolyte, which are usually 60 to 150° C. and even up to 200° C.

The voltage during the electrolysis between terminals consisting of parallel plates of equal size can easily be maintained between 0.3 and 1 volt, when the spacing of the plates is about 3 cm. Under these circumstances, the energy consumption per kg. of deposited aluminium is between 0.9 and 3 kw.-h. at 150° C.

The aluminium coatings are initially dense and compact, but as the thickness of the deposited layer increases, they become gradually granular and blistered. However, the aluminium can be deposited up to a considerable thickness without the cells being damaged by bridge formation. Within the range of layer thicknesses which are used for surface treatment, the coating is completely dense and smooth and adheres firmly, provided that the surface of the foundation material has been thoroughly cleaned. A spectroscopic examination of the deposited aluminium shows that it is at least 99.999% pure, even when ordinary foundry aluminium has been used as anode. When using quaternary ammonium compounds for the formation of the complex compounds, a large number of different electrolytes are available, by which the properties of the aluminium deposit, especially the hardness, the lustre and the grain structure can be influenced as required. For the production of aluminium coatings on metal surfaces, it may be advisable to use anodes of ultra-pure aluminium. In this case, it is unnecessary for the electrolyte to be protected in the manner described above against contamination by the anode sludge. The purity

of the aluminium produced by the process of the invention is apparent from the following experiments as well as from the spectroscopic examination:

An aluminium coating produced on a polished steel sheet as support was removed as a foil and cut into pieces about 2 cm.<sup>2</sup> square. 5 cc. of 20% hydrochloric acid was poured over one such piece. For comparison purposes, the same amount of an aluminium sheet with 99.8% aluminium was subjected to the same test. In the comparison experiment, the temperature in the acid rose within 12 minutes to 72° C. and the aluminium had then completely dissolved with violet evolution of hydrogen. The electrolytically deposited aluminium did not produce any rise in temperature and remained substantially undissolved in the hydrochloric acid for some hours.

In another similar pair of experiments, the aluminium obtained according to the process of the present invention was compared with the best quality refined ultra-pure aluminium (99.99%). It was not possible to detect a rise in temperature in either of the two cases, but the 99.99% aluminium had completely dissolved after 12 hours. The aluminium obtained by a process of the invention merely showed a decrease in weight by about 1/3.

Copper plates or copper wires which have been provided by the process of the invention with an aluminium coating a few microns thick can be kept for hours in nitric acid without it being possible to detect any corrosion of the copper by the nitric acid.

The particularly high purity of the aluminium obtained is obviously the result of the fact that all electrolytes had been prepared from distillable and also distilled organic aluminium compounds. By this means it is clearly possible for the normal impurities of the aluminium to be separated with very great effectiveness in a very simple manner.

The following examples further illustrate the invention:

#### Example 1

40 42 g. of sodium fluoride and 260 g. of aluminium triethyl are brought together under a nitrogen atmosphere and heated while stirring to 100–120° C. The solid salt dissolves and two liquid layers are obtained. The upper layer consists of practically pure triethyl and the bottom layer is an excellent electrolyte for the electrolytic deposition of aluminium and has exactly the composition NaF.2Al(C<sub>2</sub>H<sub>5</sub>)<sub>3</sub>.

#### Example 2

50 58 g. of potassium fluoride and 284 g. of aluminium diisobutyl hydride.



are heated under nitrogen and while stirring to 100° C. The salt dissolves and a homogeneous liquid is obtained which solidifies in crystalline form at about 80° C. In the melt electrolysis of this reaction product, a firmly adhering aluminium deposit is obtained on the cathode.

#### Example 3

65 58 g. of potassium fluoride are dissolved in 198 g. of aluminium triisobutyl



at about 100° C. in a nitrogen atmosphere. 85 g. of aluminium trimethyl are added to this reaction mixture while stirring and heating to 80–90° C. Two liquid layers

are formed. The upper layer is practically non-conductive to electric current, and the bottom layer has the composition  $KF \cdot Al(i-C_4H_9)_3 \cdot Al(CH_3)_3$  and is quite suitable for the electrolytic deposition of aluminium.

*Example 4*

24 g. of sodium hydride, 142 g. of aluminium diisobutyl hydride



and 114 g. of aluminium triethyl are combined in a nitrogen atmosphere and heated while stirring to 110-120°. The solid sodium hydride dissolves. The liquid reaction mixture which is formed has the composition



*Example 5*

3/4 mol (=55 g.) of potassium chloride and 1 mol (=120.5 g.) of aluminium diethyl monochloride.



are brought together under nitrogen. If the reaction mixture is heated to 100° C. the potassium chloride dissolves. A homogeneous liquid is formed which solidifies on cooling. During the melt electrolysis of this reaction product, a solid aluminium precipitate is deposited on the cathode.

*Example 6*

Tetraethyl ammonium chloride and aluminium triethyl are brought together while stirring and under nitrogen in a molar ratio of 1 mol:more than 2 mols. The solid salt dissolves and two layers are formed. The upper layer consists of practically pure aluminium triethyl. This layer is thicker in proportion as more aluminium triethyl has been used in excess. The lower layer has the exact composition  $(C_2H_5)_4NCl \cdot 2Al(C_2H_5)_3$ , and is an excellent electrolyte which is extremely suitable for the deposition of aluminium.

*Example 7*

Pyridinium methiodide is brought together with aluminium triethyl, as described in Example 6. In this case also, a yellowish to brownish liquid bottom layer is formed which is not miscible with aluminium triethyl, the said layer having the composition pyridinium methiodide.2 aluminium triethyl.

*Example 8*

Dodecyl-trimethyl-ammonium chloride is dissolved in liquid aluminium tri-n-butyl in such an amount that the molar ratio (mols) between the quaternary salt and the aluminium tri-n-butyl is greater than 1. Electrolytes of any desired composition are obtained (the quaternary salt being soluble in aluminium tri-n-butyl in all proportions) and these electrolytes deposit a good and firmly adhering precipitate on the cathode during the electrolysis.

What we claim is:

1. A process for the electrolytic deposition of aluminium upon an electrically conductive surface which comprises passing an electric current between an anode and said electrically conductive surface as a cathode through an electrolyte which consists essentially of a homogeneous melt of a true organic compound of aluminium of the general formula  $AlR(R')_2$  in which R is an alkyl group and R' is a substituent selected from the group consisting of alkyl, hydrogen and halogen, in combination with a complex compound of such aluminium compound  $AlR(R')_2$  with a compound of the formula  $MeR'$  in which Me is selected from the group consisting of alkali metals and quaternary ammonium radicals and R' has the same significance as above, said complex compound being of the

formula  $MeR'AlR(R')_2$  in which Me, R and R' have the same significance as above, the quantity of said organic compound of aluminium of the formula  $AlR(R')_2$  in said homogeneous melt being in excess of that contained in said complex compound of the formula  $MeR'AlR(R')_2$ .

2. The process of claim 1 in which said electrolyte essentially consists of a compound of said aluminium compound  $AlR(R')_2$  with said complex compound.

3. The process of claim 1 in which said electrolyte essentially consists of a mixture of said aluminium compound  $AlR(R')_2$  and said complex compound.

4. The process of claim 1 in which said electrolyte essentially consists of a solution of said aluminium compound  $AlR(R')_2$  and said complex compound.

5. The process of claim 4 in which an organic solvent which does not decompose the organic aluminium compound is the solvent for said solution.

6. The process of claim 1 in which said electrolyte essentially consists of a solution of said aluminium compound  $AlR(R')_2$  and said complex compound in which a hydrocarbon solvent is the solvent for said solution.

7. The process of claim 1 in which said electrolyte essentially consists of a solution of said aluminium compound  $AlR(R')_2$  and said complex compound in which 25 an aromatic hydrocarbon solvent is the solvent for said solution.

8. The process of claim 1 in which said electrolyte essentially consists of a solution of said aluminium compound  $AlR(R')_2$  and said complex compound in which 30 an ether is the solvent for said solution.

9. The process of claim 1 in which said electrolyte essentially consists of a solution of said aluminium compound  $AlR(R')_2$  and said complex compound in which tetrahydrofuran is the solvent for said solution.

35 10. The process of claim 1 in which said electrolyte essentially consists of a solution of said aluminium compound  $AlR(R')_2$  and said complex compound in which dioxane is the solvent for said solution.

11. The process of claim 1 in which said electrolyte 40 essentially consists of a solution of said aluminium compound  $AlR(R')_2$  and said complex compound in which a tertiary amine is the solvent for said solution.

12. The process of claim 1 in which said electrolyte 45 essentially consists of a solution of said aluminium compound  $AlR(R')_2$  and said complex compound in which dimethyl aniline is the solvent for said solution.

13. The process of claim 1 in which said electrolyte 50 essentially consists of a solution of said aluminium compound  $AlR(R')_2$  and said complex compound in which pyridine is the solvent for said solution.

14. The process of claim 1 in which said complex compound contains fluorine.

15. The process of claim 1 in which said electrolyte 55 essentially consists of a compound of the formula  $NaF \cdot 2Al(C_2H_5)_3$ .

16. The process of claim 1 in which said electrolyte essentially consists of a compound of the formula  $NaF \cdot Al(CH_3)_3 \cdot Al(C_2H_5)_3$ .

17. The process of claim 1 in which said electrolyte 60 is covered with paraffin oil.

18. The process of claim 1 in which said electrolyte is maintained under an inert gas atmosphere.

19. The process of claim 1 in which said electrolyte is maintained at a temperature between 60 and 200° C.

65 20. The process of claim 1 in which said electrolyte is maintained at a temperature between 100 and 150° C.

21. The process of claim 1 in which said anode is an aluminium anode.

22. The process of claim 1 in which said electrically 70 conductive surface is a surface of another metal.

23. The process of claim 1 in which said cathode is of shaped metal and the aluminium is deposited thereon as a coating.

**References Cited in the file of this patent****UNITED STATES PATENTS**

2,321,367 Diggin ----- June 8, 1943  
2,446,349 Wier et al. ----- Aug. 3, 1948  
2,728,718 Schickner ----- Dec. 27, 1955

**OTHER REFERENCES**

Chimica E. Industria, K. Ziegler, 1952, vol. 34, pp. 520-527.  
Studies in the Electrodeposition of Metals, Bulletin No. 206, published by University of Illinois, pp. 10 and 11.  
Z. Anorg. Chemie, F. Hein, 141, 161-226, 1924.